# EUROPEAN PATENT SPECIFICATION

(11) **EP 1 643 485 B1**
(45) Date of publication and mention of the grant of the patent: **25.11.2020**
(21) Application number: 05109052.0
(22) Date of filing: 30.09.2005
(51) Int. Cl.: G10K 11/16

(54) **Acoustically insulating material, acoustically absorbing material**
Schallisolierendes Material, Schallabsorbierendes Material,
Matériau isolant sonore, matériau absorbant sonore

(30) Priority: 01.10.2004 IT TO20040659
(43) Date of publication of application: 05.04.2006
(73) Proprietor: GUARTO - GUARNIZIONI TORINO A RESPONSABILITA' LIMITATA, 10121 Torino (IT)
(72) Inventor: CAVEZZALE, Carlo, 10122 Torino (IT)
(74) Representative: Lambacher, Michael

(56) References cited:
- GB-A- 1 471 889
- US-A- 1 823 405
- US-A- 3 649 430

## Description

The present invention relates to a sound insulating or sound proofing material.

Hereinafter, the word "sound" or alternatively "sound wave" will mean a perturbation of oscillatory nature produced by a sound source which, by propagating in elastic means, causes a variation of pressure such to be perceived by the human ear.

Hereinafter, the word "vibration" will mean an oscillatory movement of minor amplitude which can generate in a body on which a sound wave strikes.

A sound may be transmitted in the environment through the air, for example the traffic noise or the sound of a radio, or through structures, such as for example the noise of steps or objects falling on the floor.

It is known that the exposure to sounds of high intensity may be harmful for an individual's health. Furthermore, it may be dangerous in situations in which attention must be devoted to potential dangers, such as for example in industrial environments, where the noise generated by machinery makes it difficult to hear the acoustic alarm signals emitted by the machinery itself. The prolonged exposure to high intensity sounds may also cause the total or partial loss of auditory capacity.

Also in homes or offices, the presence of sounds from the outside may be cause of high discomfort and induce stress in the people who live or work there.

It has indeed been demonstrated that sound, may cause inefficiencies at work and decrease productivity, even when its intensity is not particularly high.

In particular, intermittent or low frequency sounds, such as for example the noise of office apparatuses, traffic and maintenance works, are capable of altering the concentration capacity of individuals.

Similarly, prolonged and high frequency sounds, such as for example those generated by air conditioning systems or fans, may cause physical fatigue and reduce personal performance.

Very annoying may be, for example, the transmission of sound along tubes and pipes, for example water drain pipes, or through all the elements which, inserted inside a wall, may modify its sound insulating, sound proofing and sound damping properties, such as for example electrical junction boxes and switches.

Hereinafter, the word "sound insulating property" will mean the capacity of material to reflect a sound wave; a material provided with such property will be called in turn "sound insulating".

Hereinafter, the word "sound proofing property" will mean the capacity of material to dissipate a sound wave; a material provided with such property will be called in turn "sound proofing".

It is known the reduction of noise transmitted through air or water tubes and pipes with an appropriate insulation of the same using sleeves made of multilayer sound insulating materials which, in addition to ensuring thermal insulation, also reduce the sound caused by the forced passage of air or liquids.

A type of multilayer material widely used heretofore for this purpose consists of an insulating material structure containing inside a lead plate or a bituminous septum layer. Since lead is a malleable metal and therefore provided with a plastic behaviour, the material may be modelled around a structure to be insulated thus maintaining the assumed shaped unchanged in time. For example, the material may be wrapped around a tube and therefore keep the shape of the tube contour itself.

However, as it is well known, lead is a very polluting material and is highly toxic for the people responsible for working it and those who live in environments where the lead levels are high US-A-3 649 430 discloses a laminate coupled to a polymer material core through elastomeric adhesive to dampen sound and vibration; GB-A-1 471 889 discloses a sound muffling laminate for pile drivers.

It is therefore the object of the present invention to find a material for insulating or proofing sound and vibrations which solves the problems described above.

In particular, it would be desirable to find a material which, though being mouldable around the structure to be covered and therefore being plastically deformable, does not present the toxicity of lead.

According to the present invention, such object is achieved by a material according to claim 1.

The material will now be described with reference also to the accompanying figure, which shows a non-limitative example of embodiment and shows a cross section of the material itself.

In the figure, it is indicated as a whole by 1 a material comprising a first polymeric sound insulating or sound proofing element 2 and a second metallic reticulated element 3.

The first element 2 is intimately connected to the second element 3. The second element 3 is embedded, superficially coupled, glued or fitted in.

According to the present invention, the first element 2, to have an appropriate sound insulating, sound proofing or sound damping power, presents a density higher than 1.3.

The first element 2 has an appropriate thickness to maintain a suitable flexibility of the material 1.

Preferably, the first element 2 is an elastomeric polymer selected from the group consisting of natural rubber, synthetic rubber selected from the group consisting of EPM, EPDM, butyl polymers, or mixtures of the same also vulcanised or reticulated.

Alternatively, the first element 2 is a plastic or thermoplastic polymer, preferably selected from the group consisting of polyolefins, polyamides, polyurethanes, polycarbonates, silicones, acrylate polymers, methacrylate polymers, styrenic polymers, vinyl chloride polymers, vinyl acetate polymers. In particular, , for example, LDPE (or low density polyethylene), HDPE (or high density polyethylene), PP (or polypropylene), PU (or polyurethane), EVA (or ethylene vinyl acetate), PVAC (or polyvinylacetate), SBS and SEBS, PVC (or polyvinylchloride) and CPE (or polyethylene chloride) or mixtures of the same can be used.

Alternatively, the first element 2 may also consist in a mixture of elastomeric, plastomeric, plastic or thermoplastic polymers.

According to the invention, the first element 2 is filled by means of fillers.

Preferably, the fillers are present in a percentage from 5 to 95%.

According to the invention, the fillers are selected from the group consisting of calcium carbonate, kaolin, barium sulphate, talc, dolomite, metal oxides, silica and silicates, slate, metallic powders, mica, graphite, aluminium hydroxide hydrate, magnesium hydroxide hydrate, zinc borate, titanium dioxide, carbon black, bitumen. The second element 3 comprises at least one metal or metal alloy.

Preferably, the metal is selected from the group consisting of aluminium, iron, zinc, copper, nickel, titanium, tin.

Preferably, the metal alloy is selected from the group composed of monel, bronze, steel, brass.

The second element 3 may consists in, for example, a metallic plate, for example a perforated or stretched plate, of suitable thickness to allow to be moulded around a structure to be insulated and therefore maintaining the assumed shape unchanged in time.

Preferably, the perforated or stretched plate has a thickness from 0.5 mm and 1.5 mm.

Preferably, the stretched plate presents a mesh selected from the group consisting of square, rhomboid or hexagonal mesh.

Preferably, the square mesh stretched plate presents a mesh opening from 3x3 mm to 40x40mm.

Preferably, the rhomboid mesh stretched plate presents a mesh opening from 2x1 mm to 110x40.

Preferably, the hexagonal mesh stretched plate presents a mesh opening from 2x1 mm to 110x40.

Alternatively, the second element 3 can be composed of, for example, a metallic net or cloth.

For example, the metallic nets may be electrically welded or braided.

The net and the cloth comprise wires having a diameter suitable to allow moulding the material around a structure to be insulated and therefore maintaining the assumed shaped unchanged in time, but also to make the material resistant to possible physical agents to which it may be subjected.

Preferably, the net consists of wires of diameter lower than or equal to 1.20 mm.

Preferably, the metallic net presents a mesh opening from 5x5 mm to 50x50 mm.

Preferably, the metallic cloth consists of wires of diameter lower than or equal to 3 mm.

Preferably, the metallic cloth presents a mesh number per cm² from 0.13 to 1050.

According to the invention, the material 1 also comprises at least one third sound insulating or sound proofing element 4 to increase the insulating or sound proofing provided by the material 1.

According to the invention, the third element 4 is selected from the group consisting of non-woven fabric, felt, natural cloth or fibres, for example jute or agave based, synthetic cloth or fibres, metallic fibres or films, mineral fibres, glass wool, mineral wool, expanded or closed or open cell foamed polyurethane, expanded or closed or open cell foamed melamine, closed or open cell expanded reticulated polyethylene, plasterboard.

The material 1 according to the present invention may be advantageously used for the insulating or proofing of sound and vibrations which are generated inside tubes. Indeed, such material, thanks to the presence of a metallic reticulated element, is capable of being easily moulded around the tubes therefore maintaining its shape in time.

The reticulated element allows to avoid or limit the use of devices suitable to maintain the shape of the material itself and therefore facilitates the assembly or application of the material itself.

The material according to the invention can be also advantageously used in the civil, residential and industrial building sectors for the insulation or proofing of sound, for example in walls, floors and partitioning elements in general or to damper the vibrations generated by running machinery.

Furthermore, the material according to the present invention may be advantageously used also in the railway sector, for example for the insulation of railway cars, in the yachting, cruise ship and military naval sector, for example for the insulation of cabins and bulkheads, in the industrial farming sector and in the public transport sector.

Examining the features of the material according to the present invention the advantages that the material allows to obtain are evident.

In particular, such material presents excellent insulating or proofing properties of sounds and vibrations which propagate both through the air and through structures.

Furthermore, the presence of the metallic reticulated element allows to obtain an easily mouldable material, with excellent plastic behaviour and therefore capable of deforming permanently without undergoing structural modifications and without breaking, resisting also to lacerations or perforations.

Finally, the choice of suitable polymeric elements may confer to the material, in addition to the sound insulating or sound proofing properties, also an excellent resistance to fire, water, vapour, humidity, chemical substances of various nature, impermeability to air and also heat insulating properties.

Obviously, the material may be varied by adding further elements so as to increase the sound insulating and sound proofing properties or the resistance to chemical and physical agents.

Additional features of the present invention will be apparent in the description that follows only by way of purely illustrative and non-limitative examples.

### EXAMPLES

In table 1 the features of materials made according to the present invention are indicated in detail.

**Table 1**

| **Example nr.** | **First element (layer 1)** | **Second element (layer 2)** | **Third element (layer 3)** | **Possible additional elements (layer n)** | **Connection between the first element an d the second element** | **Sequence of layers** | **Diameter of net wires or plate thickness** | **Mesh openi ng** |
|---|---|---|---|---|---|---|---|---|
| 1 | Filled EPDM | Square mesh stretched plate | Expanded PE | - | Gluing | Layer 1 -layer 2 -layer 3 | 0.8 mm | 20x20 |
| 2 | Filled EPM | Square mesh stretched plate | Embossed expanded PE | - | Gluing | Layer 1 -layer 2 -layer 3 | 0.8 mm | 20x20 |
| 3 | Filled EPDM | Square mesh stretched plate | Open cell PU | - | Gluing | Layer 1 -layer 2 -layer 3 | 0.8 mm | 20x20 |
| 4 | SBS/SEBS | Square mesh stretched plate | PVC | - | Gluing | Layer 1 -layer 2 -layer 3 | 0.8 mm | 20x20 |
| 5 | CPE | Square mesh stretched plate | Expanded melamine | - | Layer 2 embedded in layer 1 | Layer 3 -layer 1 -layer 2 -layer 3 | 0.8 mm | 20x20 |
| 6 | SBS filled with bitumen | Square mesh stretched plate | Expanded PE | Expanded PE (layer 4) | Layer 2 embedded in layer 1 | Layer 4 -layer 1 -layer 2 -layer 3 | 0.8 mm | 20x20 |
| 7 | EPDM/EPM | Zinc-plated electrically welded net | Expanded PE | - | Gluing | Layer 1 -layer 2 -layer 3 | 0.63 mm | 5 mm |
| 8 | SBS filled with bitumen | Zinc-plated electrically welded net | Open cell PU | - | Gluing | Layer 1 -layer 2 -layer 3 | 0.63 mm | 5 mm |
| 9 | EVA | Zinc-plated electrically welded net | PVC | - | Gluing | Layer 1 - layer 2 - layer 3 | 0.63 mm | 5 mm |
| 10 | PE/PP | Zinc-plated electrically welded net | Melamine | - | Gluing | Layer 1 - layer 2 - layer 3 | 0.63 mm | 5 mm |
| 11 | EPDM/EPM | Epoxy coated steel cloth | Expanded PE | - | Gluing | Layer 1 - layer 2 - layer 3 | 0.28 mm | 12x10 |
| 12 | EVA | Epoxy coated steel cloth | Non-woven - PES | Expanded PU (layer 4 and 5) | Gluing | Layer 5 - layer 3 - layer 2 - layer 1 - layer 4 | 0.28 mm | 12x10 |
| 13 | Filled PVC | Zinc-plated electrically welded net | Expanded PVC | Expanded PVC (layer 4) | Layer 2 embedded in layer 1 | Layer 4 - layer 1 - layer 2 - layer 3 | 0.63 mm | 5 mm |
| 14 | SBS | Epoxy coated steel cloth | Melamine | - | Gluing | Layer 1 - layer 2 - layer 3 | 0.28 mm | 12x10 |
| 15 | PE/PP | Steel net | PE/PP | - | Layer 2 embedded in layer 1 | Layer 1 - layer 2 - layer 3 | 0.5 mm | 20 mm |
| 16 | EPDM/EVA/P E | Zinc-plated electrically welded net | Non-woven fabric - PES | - | Gluing | Layer 1 - layer 2 - layer 3 | 0.63 mm | 5 mm |
| 17 | EPDM/EVA/P E | Epoxy coated steel cloth | - | - | Gluing | Layer 1 - layer 2 | 0.28 mm | 12x10 |
| 18 | EPM/EVA | Steel net | Expanded PU | Expanded PE (layer 4) | Gluing | Layer 4 - layer 1 - layer 4 - layer 2 - layer 4 | 0.8 mm | 40 mm |
| 19 | EVA/PE/PP | Zinc-plated triple twisted net | PP/PA/PP 20/20/20 film | - | Layer 2 embedded in layer 1 | Layer 1 - layer 2 - layer 3 | 0.70 mm | 13 mm |
| 20 | PVC | Zinc-plated electrically welded net | Expanded PVC | - | Gluing | Layer 1 - layer 2 - layer 3 | 0.65 mm | 13 mm |
| 21 | Butyl rubber | Zinc-plated electrically welded net | - | - | Embedded | Layer 1 - layer 2 | 0.65 mm | 13 mm |
| 22 | EPDM/EVA/P E | Square mesh stretched plate | Non-woven fabric - PES | Embossed expanded PE (layer 4) | Embedded | Layer 1 - layer 2 - layer 3 - layer 4 | 0.8 mm | 20x20 |

## Claims

1. Material (1) comprising at least one first polymeric sound insulating or sound proofing element (2) and at least one second metallic element (3), wherein:
- said first polymeric element (2) has a density higher than 1.3, said first element (2) being filled by means of fillers, said fillers being preferably present in a percentage from 5 to 95%, said fillers being selected from the group consisting of calcium carbonate, kaolin, barium sulphate, talc, dolomite, metal oxides, silica and silicates, slate, metallic powders, mica, graphite, aluminum hydroxide hydrate, magnesium hydroxide hydrate, zinc borate, titanium dioxide, carbon black, bitumen;
- said second metallic element (3) is reticulated; and
- the material (1) further comprises at least one third sound insulating or sound proofing element (4), said third element (4) being selected from the group consisting of non-woven fabric, felt, natural cloth or fibers, synthetic cloths or fibers, metallic fibers or films, mineral fibers, glass wool, mineral wool, expanded or closed or open cell foamed polyurethane, expanded or closed or open cell foamed melamine, closed or open cell expanded reticulated polyethylene, plasterboard;
- said first element (2) being intimately connected to said second element (2), namely said second element (3) is embedded in said first element (2) or said second element (3) is superficially coupled to said first element (2).

2. Material (1) according to claim 1, **characterized in that** said first element (2) is an elastomeric polymer selected from the group consisting of natural rubber, synthetic rubber selected from the group consisting of EPM, EPDM, butyl polymers, or mixtures of the same also vulcanized or reticulated.

3. Material (1) according to claim 1, **characterized in that** said first element (2) is a plastic or thermoplastic polymer selected from the group consisting of polyolefins, polyamides, polyurethanes, polycarbonates, silicones, acrylate polymers, methacrylate polymers, styrene polymers, vinyl chloride polymers, vinyl acetate polymers or mixtures of the same.

4. Material (1) according to any of the preceding claims, **characterized in that** said first element (2) is a mixture of elastomeric, plastomeric, plastic or thermoplastic polymers .

5. Material (1) according to any of the preceding claims, **characterized in that** said second element (3) comprises a metal selected from the group consisting of aluminum, iron, zinc, copper, nickel, titanium, tin.

6. Material (1) according to any of claims from 1 to 4, **characterized in that** said second element (3) comprises a metal alloy selected from the group consisting of monel, bronze, steel, brass.

7. Material (1) according to any of claims 5 or 6, **characterized in that** said second element (3) is a net, said net preferably consisting of wires of diameter lower than or equal to 1.20 mm, said net preferably presenting a mesh opening from 5x5 mm to 50x50 mm.

8. Material (1) according to any of claims 5 or 6, **characterized in that** said second element (3) is a cloth, said cloth preferably consisting of wires of diameter lower than or equal to 3 mm, said cloth preferably presenting a mesh number per cm² from 0.13 to 1050.

9. Material (1) according to any of claims 5 or 6, **characterized in that** said second element (3) is a stretched or perforated plate, said plate preferably presenting a thickness from 0.5 mm to 1.5 mm.

10. Material (1) according to claim 9, **characterized in that** said stretched plate presents a mesh selected from the group consisting of square, rhomboid and hexagonal mesh, said square mesh stretched plate preferably presenting a mesh opening from 3x3 mm to 40x40 mm, said rhomboid mesh stretched plate preferably presenting a mesh opening from 2xlmm to 110x40 mm, said hexagonal mesh stretched plate preferably presenting a mesh opening from 2x1 mm to 110x40 mm.

11. Use of the material (1) according to any of claims 1 to 10 for sound insulation or proofing.

## Patentansprüche

1. Material (1) umfassend wenigstens ein erstes polymerisches schalldämmendes oder schalldichtes Element (2) und wenigstens ein zweites metallisches Element (3), wobei:
- das erste polymerische Element (2) eine Dichte aufweist, die höher als 1,3 ist, das erste Element (2) mittels Füllstoffen gefüllt ist, wobei die Füllstoffe vorzugsweise in einem Prozentsatz von 5 bis 95% vorhanden sind, die Füllstoffe, von der Gruppe ausgewählt sind, die aus Calciumcarbonat, Kaolin, Bariumsulfat, Talkum, Dolomit, Metalloxiden, Kieselsäure und Silikate, Schiefer, Metallpulvern, Glimmer, Graphit, Aluminiumhydroxidhydrat, Magnesiumhydroxidhydrat, Zinkborat, Titandioxid, Ruß, Bitumen besteht;
- das zweite metallische Element (3) retikuliert ist; und
- das Material (1) ferner wenigstens eine drittes schalldämmendes oder schalldichtes Element (4) umfasst, wobei das dritte Element (4) aus der Gruppe ausgewählt ist, die aus nicht-gewebtem Stoff, Filz, Naturstoff oder -fasern, synthetischen Stoffen oder Fasern, metallischen Fasern oder Folien, Mineralfasern, Glaswolle, Mineralwolle, expandiertem oder geschlossen- oder offenzelligem geschäumten Polyurethan, expandiertem oder geschlossen- oder offenzelligem geschäumten Melamin, geschlossen- oder offenzelligem expandierten netzförmig angelegten retikulierten Polyethylen, Gipskarton besteht;
- das erste Element (2) mit dem zweiten Element (2) eng verbunden ist, nämlich das zweite Element (3) in dem ersten Element (2) eingebettet ist oder das zweite Element (3) oberflächlich mit dem ersten Element (2) gekoppelt ist.

2. Material (1) nach Anspruch 1, **dadurch gekennzeichnet, dass** das erste Element (2) ein elastomerisches Polymer ist, das aus der Gruppe ausgewählt ist, die aus Naturkautschuk, synthetischem Gummi, das aus der Gruppe ausgewählt ist, die aus EPM, EPDM, Butylpolymereren oder Gemischen derselben besteht, die auch vulkanisiert oder retikuliert sind.

3. Material (3) nach Anspruch 1, **dadurch gekennzeichnet, dass** das erste Element (2) ein plastisches oder thermoplastisches Polymer ist, das aus der Gruppe ausgewählt ist, die aus Polyolefinen, Polyamiden, Polyurethanen, Polycarbonaten, Siliconen, Acrylatpolymeren, Methacrylatpolymeren, Styrolpolymeren, Vinylchloridpolymeren, Vinylazetatpolymeren oder Gemischen der derselben bestehen.

4. Material (1) nach einem der vorhergehenden Ansprüche, **dadurch gekennzeichnet, dass** das erste Element (2) ein Gemisch aus elastomeren, plastomeren, plastischen oder thermoplastischen Polymeren ist.

5. Material (1) nach einem der vorhergehenden Ansprüche, **dadurch gekennzeichnet, dass** das zweite Element (3) ein Metall umfasst, das aus der Gruppe ausgewählt ist, die aus Aluminium, Eisen, Zink, Kupfer, Nickel, Titan, Zinn besteht.

6. Material (1) nach einem der Ansprüche 1 bis 4, **dadurch gekennzeichnet, dass** das zweite Element (3) eine Metalllegierung umfasst, die aus der Gruppe ausgewählt ist, die aus Monel, Bronze, Stahl, Messing besteht.

7. Material (1) nach einem der Ansprüche 5 oder 6, **dadurch gekennzeichnet, dass** das zweite Element (3) ein Netz ist, wobei das Netz vorzugsweise aus Drähten mit einem Durchmesser besteht, der geringer als oder gleich 1,20 mm ist, wobei das Netz vorzugsweise eine Maschenöffnung von 5x5 mm bis 50x50 mm aufweist.

8. Material (1) nach einem der Ansprüche 5 oder 6, **dadurch gekennzeichnet, dass** das zweite Element (3) ein Tuch ist, wobei das Tuch vorzugsweise aus Drähten mit einem Durchmesser besteht, der geringer als oder gleiche 3 mm ist, wobei das Tuch vorzugsweise eine Maschenzahl pro cm² von 0,13 bis 1050 aufweist.

9. Material (1) nach einem der Ansprüche 5 oder 6, **dadurch gekennzeichnet, dass** das zweite Element (3) eine gedehnte einer perforierten Platte ist, wobei die Platte vorzugsweise eine Dicke von 0,5 mm bis 1,5 mm aufweist.

10. Material (1) nach Anspruch 9, **dadurch gekennzeichnet, dass** die gedehnte Platte eine Masche aufweist, die aus der Gruppe ausgewählt ist, die aus einer quadratischen, rhomboiden und hexagonalen Masche besteht, wobei die quadratmaschige gedehnte Platte vorzugsweise eine Maschenöffnung von 3x3 mm bis 40x40 mm aufweist, die rhomboidmaschige gedehnte Platte vorzugsweise eine Maschenöffnung von von 2x1 mm bis 110x40 mm aufweist, die hexagonmaschige gedehnte Platte vorzugsweise eine Maschenöffnung von 2x1 mm bis 110x40 mm aufweist.

11. Verwendung des Materials (1) nach einem der Ansprüche 1 bis 10 zur Schalldämmung oder -dichtung.

## Revendications

1. Matière (1) comprenant au moins un premier élément polymère (2) faisant office d'isolant acoustique ou d'élément d'insonorisation et au moins un deuxième élément métallique (3), dans laquelle :
- ledit premier élément polymère (2) possède une masse volumique qui est supérieure à 1,3, ledit premier élément (2) étant rempli par l'intermédiaire de matières de remplissage, lesdites matières de remplissage étant de préférence présentes dans un pourcentage de 5 à 95 %, lesdites matières de remplissage étant choisies parmi le groupe constitué par du carbonate de calcium, du kaolin, du sulfate de baryum, du talc, de la dolomite, des oxydes métalliques, de la silice et des silicates, du schiste, des poudres métalliques, du mica, du graphite, de l'hydrate d'hydroxyde d'aluminium, de l'hydrate d'hydroxyde de magnésium, du borate de zinc, du dioxyde de titane, du noir de carbone, du bitume ;
- ledit deuxième élément métallique (3) est réticulé ; et
- la matière (1) comprend en outre au moins un troisième élément (4) faisant office d'isolant acoustique ou d'élément d'insonorisation, ledit troisième élément (4) étant choisi parmi le groupe constitué par de l'étoffe non tissée, du feutre, des fibres naturelles ou des tissus naturels, des fibres ou des tissus synthétiques, des fibres ou des films métalliques, des fibres minérales, de la laine de verre, de la laine minérale, du polyuréthane transformé en mousse du type expansé ou à alvéoles fermées ou ouvertes, de la mélamine transformée en mousse du type expansé ou à alvéoles fermées ou ouvertes, du polyéthylène réticulé expansé du type à alvéoles fermées ou ouvertes, du placoplâtre ;
- ledit premier élément (2) étant intimement relié audit deuxième élément (2) ; plus précisément, ledit deuxième élément (3) est incorporé dans ledit premier élément (2) ou bien ledit deuxième élément (3) est couplé en surface audit première élément (2).

2. Matière (1) selon la revendication 1, **caractérisée en ce que** ledit premier élément (2) représente un polymère élastomère qui est choisi parmi le groupe constitué par du caoutchouc naturel, du caoutchouc synthétique choisi parmi le groupe constitué par du EPM, du EPDM, des polymères de type butyle, ou des mélanges des polymères en question également à l'état vulcanisé ou à l'état réticulé.

3. Matière (1) selon la revendication 1, **caractérisée en ce que** ledit premier élément (2) représente un polymère plastique ou thermoplastique qui est choisi parmi le groupe constitué par des polyoléfines, des polyamides, des polyuréthanes, des polycarbonates, des silicones, des polymères d'acrylate, des polymères de méthacrylate, des polymères de styrène, des polymères de chlorure de vinyle, des polymères d'acétate de vinyle, ou des mélanges des polymères en question.

4. Matière (1) selon l'une quelconque des revendications précédentes, **caractérisée en ce que** ledit premier élément (2) représente un mélange de polymères élastomères, plastomères, plastiques ou thermoplastiques.

5. Matière (1) selon l'une quelconque des revendications précédentes, **caractérisée en ce que** ledit deuxième élément (3) comprend un métal qui est choisi parmi le groupe constitué par de l'aluminium, du fer, du zinc, du cuivre, du nickel, du titane, de l'étain.

6. Matière (1) selon l'une quelconque des revendications 1 à 4, **caractérisée en ce que** ledit deuxième élément (3) comprend un alliage métallique qui est choisi parmi le groupe constitué par du monel, du bronze, de l'acier, du laiton.

7. Matière (1) selon l'une quelconque des revendications 5 ou 6, **caractérisée en ce que** ledit deuxième élément (3) représente un treillis, ledit treillis étant de préférence constitué par des fils dont le diamètre est inférieur ou égal à 1,20 mm, ledit treillis présentant de préférence une ouverture de maille de 5x5 mm à 50x50 mm.

8. Matière (1) selon l'une quelconque des revendications 5 ou 6, **caractérisée en ce que** ledit deuxième élément (3) représente une étoffe, ladite étoffe étant de préférence constituée par des fils dont le diamètre est inférieur ou égal à 3 mm, ladite étoffe présentant de préférence un nombre de mailles par cm² de 0,13 à 1050.

9. Matière (1) selon l'une quelconque des revendications 5 ou 6, **caractérisée en ce que** ledit deuxième élément (3) représente une plaque tendue ou perforée, ladite plaque présentant de préférence une épaisseur de 0,5 mm à 1,5 mm.

10. Matière (1) selon la revendication 9, **caractérisée en ce que** ladite plaque tendue présente une maille choisie parmi le groupe constitué par une maille carrée, rhomboïde et hexagonale, ladite plaque tendue possédant une maille carrée présentant de préférence une ouverture de maille de 3x3 mm à 40x40 mm, ladite plaque tendue possédant une maille rhomboïde présentant de préférence une ouverture de maille de 2x1 mm à 110x40 mm, ladite plaque tendue possédant une maille hexagonale présentant de préférence une ouverture de maille de 2x1 mm à 110x40 mm.

11. Utilisation de la matière (1) selon l'une quelconque des revendications 1 à 10, pour l'isolation acoustique ou l'insonorisation.
